

W. H. BRISTOL.  
ART OF MELTING METALS.  
APPLICATION FILED DEC. 24, 1918.

1,315,206.

Patented Sept. 9, 1919.



Inventor  
William H. Bristol  
By his Attorney  
Fred K. Buetta

# UNITED STATES PATENT OFFICE.

WILLIAM H. BRISTOL, OF WATERBURY, CONNECTICUT, ASSIGNEE TO THE BRISTOL COMPANY, OF WATERBURY, CONNECTICUT, A CORPORATION OF CONNECTICUT.

## ART OF MELTING METALS.

1,315,206.

Specification of Letters Patent. Patented Sept. 9, 1919.

Application filed December 24, 1918. Serial No. 282,132.

*To all whom it may concern:*

Be it known that I, WILLIAM H. BRISTOL, a citizen of the United States, and a resident of Waterbury, in the county of New Haven and State of Connecticut, have invented certain new and useful Improvements in the Art of Melting Metals, of which the following is a specification.

The invention relates to the melting and alloying of metals, and is directed more particularly to the prevention of oxidation of the same during the melt.

It is known to provide for this purpose the gaseous products of combustion of the fuel employed to effect the melt, but difficulty is experienced in properly directing such products over the metal, the action is not satisfactory nor efficient, and, furthermore, the products of combustion tend to contaminate the metal by introducing undesirable foreign matter. It is the object of the present invention to provide and so direct a suitable and economical medium that the highly desirable result of practically obviating oxidation is attained without these detrimental features being present, said method effecting great saving and permitting of the carrying on of the melting in a more rapid and safe manner. To this end, there is directed over the surface of the metal, to provide a suitable envelop to exclude the air, a stream of steam, preferably dry and superheated, and in such manner as to afford a continuous supply of fresh steam and without interfering with the simultaneous operation of the various stirring devices required for the proper mixing of the metal or metals.

The nature of the invention will be best understood when described in connection with the accompanying drawings, in which—

Figure 1 is a vertical section through one type of furnace to which the new process may be applied.

Figs. 2 and 3 illustrate, respectively, a transverse and a longitudinal section of a resistor type of electric furnace, illustrating one form of electric furnace to which the process may be applied.

Similar characters of reference designate corresponding parts throughout the several views.

Referring to the drawings, and more particularly to Fig. 1 thereof, 10 designates a

suitable furnace provided with a grate 11, and flue 12, the former being designed to support a combustible such as coal 13, and the latter to remove the products of combustion. The furnace is designed to be closed by means of a removable top or cover 14 which may be moved over the top of the furnace to provide an opening 15, or the latter may be formed directly in the said cover. Opening 15, moreover, will permit of the introduction of the usual and well-known stirring and like instruments (not shown) employed in the melting and alloying.

Upon the bed of coal 13 rests a suitable retainer as the pot or crucible 16 for the metal or metals 17 to be melted or alloyed, all of which is well understood and forms no particular part of the present invention.

The invention relates more particularly to the provision of a suitable non-oxidizing medium to envelop the molten metal 17, thereby excluding access of air, as well as the products of combustion which might contaminate the metal as by the introduction of carbonaceous or other foreign matter. To this end, there is introduced over or into the crucible 16, steam, which is preferably in dry and superheated condition, and which will introduce no objectionable by-products. Even should the stream contain a certain small percentage of moisture, no difficulty would be experienced as the moisture would be immediately converted into steam. The supply of this steam may be economically obtained and is readily controlled, the same being furnished, generally, in a continuous stream during the period of melt and particularly during the introduction of an alloying metal. The supply of steam may be conveniently introduced through the opening 15 as by a suitable thermally insulated pipe or nozzle 18 which, as aforesaid, may be directed into the furnace space 19 or into the upper portion of the crucible 16, the spent steam being drawn off through the flue 12.

Although the invention has been shown in connection with only one type of fuel fired furnace, it is to be understood that the same is applicable to various well-known types, also to the electric type of furnace, more particularly shown in Figs. 2 and 3. As an example of this form of furnace, a resistor type is shown, the same comprising

a lower semi-cylindrical portion 25 designed to retain the metal 26, and over which is fitted a cover or top 27 similarly shaped. This top affords an opening 28 to receive an 5 inlet pipe 29 for delivering steam to the interior of the furnace, and an outlet 30 for the spent steam through which, also, there may be introduced suitable stirring and like 10 well-known instruments (not shown) and employed in the melting and alloying. The interior is heated through a suitable resistor member such as a carbon rod 31 which is mounted, in any convenient and well-known manner. This form affords a very satisfactory furnace in that the temperature thereof is readily controlled, the heat being reflected from the inner surface of the cover 27 to the metal 26; and, furthermore, the steam will not have a tendency to extinguish the 15 source of heat. The steam, moreover, is beneficial not only with respect to the materials being melted, but also in preventing the oxidation of the resistor member 31, and consequently prolonging the life of same 20 and reducing the expense of operation. For the preparation of alloys, particularly brass in its various proportions, a furnace—either electric or fuel heated—thus secured against oxidation of its melt is of the greatest value.

## 1 claim:

1. In the melting of metals: the process of preventing oxidation thereof, which consists in providing over the surface of same an envelop of steam.
2. In the melting of metals: the process of preventing oxidation thereof, which consists in providing over the surface of same an envelop of dry steam.
3. In the melting of metals: the process of preventing oxidation thereof, which consists in providing over the surface of same an envelop of superheated steam.
4. In the melting of metals: the process of preventing oxidation thereof, which consists in excluding air therefrom, by directing a stream of steam over the surface thereof.
5. The method of preventing oxidation of metal being melted in a furnace having a gas outlet and an opening for the insertion of suitable stirring apparatus, which consists in directing a stream of steam through said opening while the metal is being melted, and causing the spent steam to leave through the said outlet.

Signed at Waterbury in the county of 55  
New Haven and State of Connecticut this  
21<sup>st</sup> day of December, A. D. 1918.

WILLIAM H. BRISTOL.